

May 4, 1965

M. J. BROOKS ET AL

3,181,944

ZINC CALCINE FOR HYDROMETALLURGICAL PROCESS

Filed May 7, 1962



INVENTORS:  
MAXWELL J. BROOKS  
ROBERT I. NEWMAN

BY  
*Alvin J. Gettman*  
ATTORNEY

1

3,181,944  
ZINC CALCINE FOR HYDROMETALLURGICAL  
PROCESS

Maxwell J. Brooks, New York, N.Y., and Robert I. Newman, Allendale, N.J., assignors to Allied Chemical Corporation, New York, N.Y., a corporation of New York

Filed May 7, 1962, Ser. No. 192,661  
4 Claims. (Cl. 75—9)

This invention relates to the oxidation and desulphurization of zinc sulfide ores and more particularly refers to a new and improved process for calcining zinc sulfide concentrates with high iron content to produce a zinc calcine for hydrometallurgical treatment and concomitantly high strength  $\text{SO}_2$  gas for conversion into  $\text{H}_2\text{SO}_4$ .

Zinc sulfide ores used for production of metallic zinc are usually flotation concentrates which are finely ground to free the individual ore from gangue particles. The zinc content will range from about 45—55% and sulfur from 27—36% with iron present in quantities ranging from about 1% to 15%. The roasted zinc oxide, usually termed calcine, is employed to convert it to zinc metal by two distinct methods (a) pyrometallurgical process and (b) hydrometallurgical process. If the calcine is to be converted by a pyrometallurgical process such as retort distillation, the quality of the roasted zinc oxide is usually not as critical. Fine calcine is usually agglomerated or sintered prior to retorting and residual sulfur content of calcine, which can supply a portion of the fuel, is eliminated during sintering. Furthermore, soluble zinc content of calcine is of no concern in pyrometallurgical operations.

In hydrometallurgical processes, calcine quality is of major importance and maximum solubility of the zinc content of the calcine in leach liquor is essential. Small increases in solubility of the calcine in leach liquor has a profound effect on the efficiency and economics of the process—an increase in solubility of 2% may reflect a saving of a quarter of a million dollars a year for a zinc plant of average size. In addition certain impurities normally produced in roasting materially reduce the yield and hamper and complicate the electrolytic refining. From the foregoing it will be evident that the quality of the calcine produced by roasting has an important bearing on the subsequent conversion of the calcine by hydrometallurgical process. The present invention is particularly directed to producing a calcine suitable for hydrometallurgical refining and processes requiring a high quality calcine product.

An object of the present invention is to provide an efficient process for calcining zinc sulfide ores containing iron to produce sulfur dioxide and calcine eminently suitable for conversion to metallic zinc by hydrometallurgical process. Another object of the present invention is to provide a process for roasting iron zinc concentrates to produce a calcine with lower sulfide and sulfate sulfur and at the same time higher soluble zinc. Other objects and advantages will be apparent from the following description and accompanying drawing.

In hydrometallurgical processes for production of metallic zinc, zinc calcine is leached with leach liquor which is an aqueous solution of sulfuric acid, the latter reacting with the zinc oxide in the calcine to form zinc sulfate. This liquor is then subjected to electrolysis to deposit zinc metal and form sulfuric acid which latter is recirculated as leach liquor for leaching additional zinc calcine. The quality of zinc calcine for hydrometallurgical process is most important to the success of the operation. The quality of calcine is determined by (a) concentration of zinc sulfide ( $\text{ZnS}$ ), (b) concentration of zinc sulfate ( $\text{ZnSO}_4$ ), (c) concentration of ferrite ( $\text{ZnO} \cdot \text{Fe}_2\text{O}_3$ ) which factors in turn materially affect the solubility of zinc con-

2

tent of the calcine in leach liquor. Zinc sulfide in the calcine is insoluble in the leach liquor and represents a yield loss. In practice the maximum amount of zinc sulfide in the calcine considered tolerable is 0.6 percent and of course any reduction in zinc sulfide below this maximum value represents material gain. Zinc sulfate is soluble in the leach liquor, but, the ratio of zinc oxide to sulfate in the calcine is limited by requirements of the leaching and electrolytic circuits. Should the sulfate content of the calcine exceed a limit of about 2.0 percent, purging of the leach liquor will be required, also entailing a loss in zinc yield. A further complication is introduced by the presence of iron in the ore feed. Zinc oxide and ferric oxide in intimate contact react to form acid insoluble zinc ferrites ( $\text{ZnO} \cdot \text{Fe}_2\text{O}_3$ ). The loss in zinc due to insoluble zinc ferrites is represented in the industry as the ferritization ratio defined as the weight of zinc rendered insoluble by a unit weight of iron. To illustrate these values reference is made to the article "Suspension Roasting of Zinc Concentrates" by R. E. Eyre, page 592, Canadian Mining & Metallurgical Bulletin, vol. 54, No. 592, August 1961, wherein the ferritization ratio of prior art method is given as 0.522 and emphasis is placed on the fact that the author reports on an operation which succeeded in reducing the ferritization ratio to 0.46. Obviously a process which obtains even further reduction in the ferritization ratio represents a marked improvement in the art. From the foregoing it will be evident that the quality of zinc calcine for use in hydrometallurgical processes is complicated by several factors and reflects itself materially in the operation of the hydrometallurgical process.

Roasting of sulfide ores is an old art and in fact roasting of ore in a fluidized bed with entrainment of fines was disclosed more than 80 years ago. However roasting of zinc sulfide ores containing iron for use in hydrometallurgical processes presents peculiar and difficult problems in that the resultant zinc calcine inherently contains impurities which either require separate treatment for removal of these impurities or place a material cost burden on the recovery of zinc by the hydrometallurgical process. We have carried out extensive experimentation for the purpose of calcining zinc sulfide ores contaminated with iron to produce a zinc calcine which is lower in the undesirable impurities namely, zinc sulfide, zinc sulfate and ferrites, thereby increasing the solubility of the zinc content of the calcine and increasing the yield of recoverable zinc. In the course of our investigation on calcination of zinc sulfide ores we found that conditions which tended to minimize formation of one impurity had the reverse effect on other impurities. More specifically we found that oxidation of zinc sulfide in air at relatively low temperatures resulted in zinc sulfate as the principal product rather than zinc oxide. Also we found it necessary that adequate temperature level be maintained to effect as complete desulphurization as possible which conditions would indicate the need of high temperature and long time to accomplish complete roasting operation. On the other hand we found that the rate of formation of ferrite increases with temperature and time of contact. Accordingly, we directed our efforts to calcination operation conditions wherein the temperature was sufficiently high to effect substantially complete desulphurization with minimum formation of zinc sulfate and the time of contact low to retard ferrite formation. But even under these conditions it was found that undesirable amounts of zinc sulfate were formed. Further investigation showed that this deleterious effect took place outside of the calcination zone. Thus, it will be seen that calcination of zinc sulfide ores containing iron to produce a calcine particularly suitable for a hydro-

metallurgical process is complicated and dependent upon several factors.

In accordance with the present invention we have produced from zinc sulfide ore containing iron a zinc calcine eminently suitable for hydrometallurgical process and containing only minor amounts of zinc sulfide, zinc sulfate and ferrite with high solubility of the zinc content of the calcine in leach liquor by maintaining at a temperature within the range of 1500-1650° F., preferably 1550-1600° F. a fluidized bed containing particles of partially roasted ore finer than about 100 mesh size and particles of substantially completely roasted ore larger than about 100 mesh size, introducing iron containing zinc sulfide ore containing particles finer than about 100 mesh and coarser than about 100 mesh into the fluidized bed at a point below the top surface of the fluidized bed and about 6 inches to 3 feet above the bottom surface of the bed, passing an oxygen containing gas, preferably air, in an amount at least sufficient to convert the sulfide ore to the corresponding oxide up through the bed to maintain the bed in fluidized condition and to partially oxidize the feed sulfide ore and to entrain and carry out of the fluidized bed partially roasted particles of ore finer than about 100 mesh, introducing gas above the top surface of the fluidized bed for control of temperature in the free space above the bed, passing the suspension of partially roasted feed ore in gas from the top of the bed into a free space thereabove having a volume at least seven times preferably 10-20 times the volume of the fluidized bed, passing the partially roasted ore suspended in the gas through the free space to effect substantially complete oxidation of the sulfide ore to the corresponding oxide, maintaining the temperature of the free space thereabove within the range of 1500-1800° F. preferably within the range of 1650-1750° F., discharging the substantially completely roasted ore and gas from the free space, separating the roasted ore particles from the gas i.e. at least about 75 percent preferably in excess of 90 percent, while maintaining a temperature of at least 1450° F. preferably within the range of 1500-1700° F., prior to and during separation of the roasted ore particles from the gas, discharging the separated roasted particles from the separator, thereafter cooling the gas e.g. by a waste heat boiler and recovering the remainder of the fine particles of dust in the gas e.g. by hot gas electrostatic precipitator. The temperature in the fluid bed and the free space above it may be controlled by any suitable cooling means, since the reaction is highly exothermic. A convenient method of controlling the temperature of the fluid bed is by the introduction of a liquid such as water or waste acid and the temperature of the free space above the bed may be controlled by recycling cooler gas or by spraying liquid in to the top of the reaction chamber or a combination of these methods.

The accompanying drawing diagrammatically illustrates one method of carrying out the operation of the present invention.

Referring to ore storage bin 1 in the drawing, zinc sulfide ores, the charge to the process, used for production of metallic zinc are usually concentrates which can range from about 40-95 percent finer than 100 mesh with the remainder generally coarser than 100 mesh and usually a maximum size of about  $\frac{1}{4}$  inch. The zinc content will range from 45-55 percent and sulfur from about 27-36% or more. Iron may be present in quantities ranging from about 1 percent to about 15-20 percent. Other impurities such as copper, lead and cadmium may also be present. The ore feed from bin 1 passes down through line 2 and is fed by means of screw 3 directly into fluid bed 4 at a point below the upper surface of the fluid bed but at a point of about  $\frac{1}{2}$ -3 feet above the lower surface of the bed. The fluid bed is supported on distributor plate 5 which may be a horizontal plate having perforations to permit the passage of air up through the plate. Bed 4 is composed of solid particles ranging from

larger particles of roasted ore up to about  $\frac{1}{4}$  inch size to fine particles below 100 mesh of partially roasted ore. Oxygen containing gas, preferably air, for fluidizing and combustion is introduced by means of fan 6 through line 7 into wind box 8 below distributor plate 5 and then passes upwardly through plate 5 and bed 4.

As the feed ore enters bed 4 at a point a short distance above the bottom of the bed it is partially roasted and the fine particles below about 100 mesh of partially roasted ore are swept out and carried into the free space above the bed. The larger particles of ore above about 100 mesh are retained in the bed where they are substantially completely roasted. Complete oxidation of the finely divided ore particles in the fluid bed 4 need not be attempted. The temperature in the fluid bed should be at least 1500° F. and should not exceed 1650° F. Temperatures below 1500° F. were found to induce the formation of zinc sulfate and temperatures above 1650° F. in the bed may cause localized hot spots which tend to increase ferrite formation. Since the reaction is highly exothermic there is a tendency for the temperature to rise to an undesired height and water or waste acid entering through line 9 may be introduced in regulated amounts for controlling the bed temperature. The air passes up through the bed 4 at a moderate velocity, about  $2\frac{1}{2}$ - $3\frac{1}{2}$  feet per second, sufficient to fluidize the bed and carry the fine particles above the bed. Extremely high velocities are undesirable as they introduce excessive amounts of air which dilutes the concentration of  $\text{SO}_2$  in the discharge gas. Also high velocity gas would entrain and carry particles larger than about 100 mesh with possible loss of fluidization. Roaster 11 is a vertical chamber wherein the reaction takes place with as previously described a distributor plate 5 near the bottom on which is supported a fluid bed 4 and above which is a free space 12 wherein desulphurization is substantially completed. In our investigation we found that the relative height of the free space 12 compared to the height of the fluid bed 4 was important and to obtain good results the free space should have a height at least 7 times the height of the fluid bed preferably 10 to 20 times the height of the fluid bed. Merely as illustrative, a roaster 20 feet in diameter and 50 feet high would have a height of fluid bed of 5 feet and a free space above the fluid bed or 45 feet or a ratio of 9:1. The entrained partially burned ore solids in the gas pass upwardly from the top of fluid bed 4 through the free space 12 wherein oxidation continues. The temperature in the free space 12 should be within the range of 1500-1800° F. and preferably within the range of 1650-1750° F. Temperatures above 1800° F. favor ferrite formation and should be avoided. The temperature in free space 12 should desirably be above 1650° F. to facilitate complete desulphurization and minimize zinc sulfide. The temperature in free space 12 may be maintained higher than bed 4 because in free space 12 the particles are in dispersed condition and undesirable localized hot spots will not occur whereas in bed 4 under such higher temperatures there will be such localized hot spots due to the close proximity of the particles. The temperature in free space 12 may be regulated by introduction of water or waste acid entering through line 13 or by cooled recycle gas entering roaster 11 through line 14. The gas entering free space 12 through line 14 serves to cool the free space and, particularly in view of the great height of the free space, aids in carrying the fine particles up through the free space and out of the reaction zone. Velocity of gas in the free space due to introduction of additional gas and/or liquid coolant there is appreciably higher than in fluid bed 4 and is of the order of about 4-10 feet per second. As previously mentioned the ore feed introduced into roaster 11 by means of screw 3 contains some larger size particles usually 5 to 25 percent which particles are too large to be entrained by the up-rising air passing through the bed and therefore accu-

mulate in fluid bed 4. This accumulation of roasted ore may be discharged from the bed by means of screw 15 through line 16 either continuously or intermittently.

Gases and suspended roasted particles are released from the top of roaster 11 through flue 17 which is insulated to minimize heat loss and temperature drop, and then discharge into hot dust collector 18 which may be a centrifugal dust collector of a conventional cyclone type wherein substantially all the solid particles usually 85-90 percent are separated from the gases and discharged from the bottom of hot dust collector 18 by means of screw 19 through line 21. It is most important that separation of the bulk of dust from the gases take place at a high temperature, above 1450° F. and without prior cooling before and during separation to a temperature below 1450° F. or else the quality of the product will be appreciably deteriorated. To insure that the temperature in the hot dust collector 18 remains above 1450° F. preferably at a temperature of 1500-1700° F., the dust collector may be heated externally or be heavily insulated.

Gases substantially free of suspended solids but containing minor amount of fine dust discharge from the top of dust collector 18 through line 22 where they are introduced into conventional waste heat boiler 23 for the purpose of cooling the gases generally to a temperature about 500-700° F. and for utilizing the sensible heat in the gases to generate steam in the waste heat boiler which is bled from the waste heat boiler through line 24. Any small amount of fines which deposit in waste heat boiler 23 may be discharged through line 25 and directed by means of screw 26 and line 27 to storage. The cooled gases released from waste heat boiler through line 28 are forced by means of fan 29 through conventional hot gas electrostatic precipitator 31 to remove the last traces of fine particles of dust entrained in the gas which dust is discharged through line 32, screw 33 and line 34. The purified cooled gas containing SO<sub>2</sub> is directed via line 35 to conventional contact process for conversion to H<sub>2</sub>SO<sub>4</sub>. A portion of the cooled gas discharging through line 28 from waste heat boiler 23 may be returned by means of fan 36 through line 14 to free space 12 of roaster 11. The calcine discharging through lines 16, 21, 27 and 34 may be separately collected or may be combined and pass through line 37 into cooler 38 wherein the calcine is cooled to a temperature of about 200° F. and then directed via line 39 to the leaching operation for the hydrometallurgical process.

The below examples illustrate the present invention.

#### Example I

Zinc sulfide concentrates were burned in a roaster with an inside diameter of 5 feet and approximately 50 feet high with a distributor grate mounted in the base of the burner. Air for fluidizing and combustion was introduced into a wind box below the distributor plate through a flue from a blower. Ore was introduced into the burner at a single point 1 foot above the grate into a bed of prior roasted calcine. A discharge outlet for periodic discharge of bed roasted calcine was located about 14 inches above the distributor grate about 180° from the ore inlet. Water for controlling bed temperature was introduced through a ½ inch pipe located 4 feet above the grate. Cooled recycled gas was introduced into the suspension zone through a single 6 inch nozzle 9 feet 3 inches above the grate. Additional water for suspension zone temperature control was introduced through a single spray nozzle 12.5 feet above the grate.

Process gases and suspended calcined particles were removed from the top of the roaster through an insulated horizontal flue to an insulated dust collector which had an efficiency of 85-95% with a 4 inch to 6 inch H<sub>2</sub>O pressure drop. The gases were piped to a waste heat boiler of a conventional sulfuric acid plant and through an electrostatic precipitator, where remaining fine suspended dust particles were removed. A portion of the cooled

75

dust-free gases passed through a blower, and recycled back to the main burner for suspension zone temperature control.

5 Calcines from the burner, dust collector and electrostatic precipitator were collected and weighed. They were then composited on a weight basis for subsequent leaching tests.

10 Using the above equipment, a zinc flotation concentrate assaying 50.2 percent Zn, 13.4 percent Fe and 35.7 percent S dry basis, containing 2.8 percent moisture, and 48.1 percent -325 mesh, 90 percent -100 mesh and 10 percent +100 mesh was fed into the burner at a rate of 22.3 lbs./minute over an 18 hour period. Air was fed up through the grate at the rate of 905 s.c.f.m. into a 51 inch fluidized bed of 72#/c.f. density. Bed temperature was maintained at 1575° F. by injection of 6# H<sub>2</sub>O/minute into the fluid bed. Recycled gas at the rate of 200 c.f.m. was introduced into the suspension zone. Suspension zone temperature increased from 1575° F. 8 feet above the base plate to a maximum of 1730° F. 29 feet and 1715° F. 45 feet above the base. Overall pressure drop through the 51 inch fluid bed was 135 inch H<sub>2</sub>O and 5.5 inch H<sub>2</sub>O through the dust collector.

15 20 25 30 35 40 45 50 55 60 65 70 75

4 percent of the resulting calcine was discharged from the fluid bed, 6 percent from the electrostatic precipitator and the balance of 90 percent from the hot dust collector. Composite calcine contained 60.2 percent zinc, 16.4 percent Fe, 0.2 percent sulfide sulfur, 0.6 percent sulfate sulfur and a ferritization ratio of 0.312. Soluble zinc as determined by a standard leach test was 55.1 percent or 91.4 percent of total zinc content. Free oxygen content of the discharge gas at burner exit was 5.5 percent.

#### Example II

35 40 45 50 55 60 65 70 75

In the same equipment as in Example I, zinc flotation concentrate containing 55.0 percent Zn, 8.9 percent Fe and 33.4 percent S, dry basis, containing 6.6 percent moisture and 88.2 percent -325 mesh 95 percent -100 mesh and 5 percent +100 mesh was fed into the burner at a rate of 26.5#/minute over a 28 hour period. Air was fed up through the grate at the rate of 880 s.c.f.m. into a 45 inch fluidized bed of 75#/c.f. density. Bed temperature was maintained at 1575° F. by injection of 3# H<sub>2</sub>O/minute into the bed. Recycle gas flow was 490 s.c.f.m. into the suspension zone. Suspension zone temperatures were 1575° F. 8 feet above the grate, a maximum of 1725° F. at 29 feet above the grate and 1670° F. at the dust collector inlet. Overall pressure drop through the 45 inch bed was 125 inch H<sub>2</sub>O and 5.5 inch across the dust collector. Calcine distribution was 4 percent from the bed, 6 percent from the electrostatic precipitator and 90 percent from the dust collector. Composite calcine contained 65.9 percent total Zn, 61.8 percent soluble zinc, 10.8 percent Fe, 0.10 percent sulfide sulfur, 0.62 percent sulfate sulfur and a ferritization ratio of 0.380, with a leach efficiency of 93.4 percent.

Although certain preferred embodiments of the invention have been disclosed for purpose of illustration, it will be evident that various changes and modifications may be made therein without departing from the scope and spirit of the invention.

We claim:

1. A process for the production of zinc calcine characterized by low ferritization ratio, low zinc sulfide, low zinc sulfate and high solubility of the zinc content of the calcine in leach liquor, which comprises maintaining at a temperature within the range of 1500-1650° F. a fluidized bed containing particles of partially roasted ore finer than 100 mesh and particles of substantially completely roasted ore larger than 100 mesh, introducing iron containing zinc sulfide ore containing particles finer than 100 mesh and coarser than 100 mesh into the fluidized bed at a point below the top surface of the fluidized bed and about ½-3 feet above the bottom surface of the bed, passing an oxygen containing gas in an amount at least

sufficient to convert the sulfide ore to the corresponding oxide up through the bed to maintain the bed in fluidized condition and to partially oxidize the feed sulfide ore and to entrain and carry out of the fluidized bed partially roasted particles of ore finer than about 100 mesh, passing the suspension of partially roasted feed ore in gas from the top of the bed into a free space thereabove having a height at least seven times the height of the fluidized bed, passing the partially roasted ore suspended in the gas through the free space to effect substantially complete oxidation of the sulfide ore to the corresponding oxide, maintaining the temperature of the free space thereabove within the range of 1500-1800° F., discharging the substantially completely roasted ore and gas from the free space, separating roasted ore particles from the gas while maintaining a temperature of at least 1450° F. prior to and during separation of the roasted ore particles from the gas, discharging the separated roasted particles from the separator and discharging the gas from the separator.

2. A process for the production of zinc calcine characterized by low ferritization ratio, low zinc sulfide, low zinc sulfate and high solubility of the zinc content of the calcine in leach liquor, which comprises maintaining at a temperature within the range of 1550-1600° F. a fluidized bed containing particles of partially roasted ore finer than 100 mesh and particles of substantially completely roasted ore larger than 100 mesh, introducing iron containing zinc sulfide ore containing particles finer than 100 mesh and coarser than 100 mesh into the fluidized bed at a point below the top surface of the fluidized bed and about 1/2-3 feet above the bottom surface of the bed, passing an oxygen containing gas in an amount at least sufficient to convert the sulfide ore to the corresponding oxide up through the bed to maintain the bed in fluidized condition and to partially oxidize the feed sulfide ore and to entrain and carry out of the fluidized bed partially roasted particles of ore finer than about 100 mesh, introducing recycled cooled gas above the top surface of the fluidized bed, passing the suspension of partially roasted feed ore in gas from the top of the bed into a free space thereabove having a height ten to twenty times the height of the fluidized bed, passing the partially roasted ore suspended in the gas through the free space to effect substantially complete oxidation of the sulfide ore to the corresponding oxide, maintaining the temperature of the free space thereabove within the range of 1600-1750° F., discharging the substantially completely roasted ore and gas from the free space, separating roasted ore particles from the gas while maintaining a temperature of 1500-1700° F. prior to and during separation of the roasted ore particles from the gas, discharging the separated roasted particles from the separator and discharging the gas from the separator.

3. A process for the production of zinc calcine characterized by low ferritization ratio, low zinc sulfide, low zinc sulfate and high solubility of the zinc content of the calcine in leach liquor, which comprises maintaining at a temperature within the range of 1550-1600° F. a fluidized bed containing particles of partially roasted ore finer than 100 mesh and particles of substantially completely roasted ore larger than 100 mesh, introducing iron containing zinc sulfide ore containing particles finer than 100 mesh and coarser than 100 mesh into the fluidized bed at a point below the top surface of the fluidized bed and about 1/2-3 feet above the bottom surface of the bed, passing an oxygen containing gas in an amount at least sufficient to convert the sulfide ore to the corresponding oxide up through the bed to maintain the bed in fluidized condition and to partially oxidize the feed sulfide ore and to entrain and carry out of the fluidized bed partially roasted particles of ore finer than about 100 mesh, passing the suspension of partially roasted feed ore

in gas from the top of the bed into a free space thereabove having a height ten to twenty times the height of the fluidized bed, passing the partially roasted ore suspended in the gas through the free space to effect substantially complete oxidation of the sulfide ore to the corresponding oxide, maintaining the temperature of the free space thereabove within the range of 1600-1750° F., controlling the temperature of the fluid bed by the introduction of water directly into the fluid bed and the temperature of the free space above the bed by recycling cooler gas into the free space, discharging the substantially completely roasted ore and gas from the free space, separating at least 90 percent of the roasted ore particles from the gas while maintaining a temperature within the range of about 1500-1700° F. prior to and during separation of the roasted ore particles from the gas, discharging the separated roasted particles from the separator, and discharging the gas from the separator.

4. A process for the production of zinc calcine characterized by low ferritization ratio, low zinc sulfide, low zinc sulfate and high solubility of the zinc content of the calcine in leach liquor, which comprises maintaining at a temperature within the range of 1550-1600° F. a fluidized bed containing particles of partially roasted ore finer than 100 mesh and particles of substantially completely roasted ore larger than 100 mesh, introducing iron containing zinc sulfide ore containing particles finer than 100 mesh and coarser than 100 mesh into the fluidized bed at a point below the top surface of the fluidized bed and about 1/2-3 feet above the bottom surface of the bed, passing an oxygen containing gas in an amount at least sufficient to convert the sulfide ore to the corresponding oxide up through the bed to maintain the bed in fluidized condition and to partially oxidize the feed sulfide ore and to entrain and carry out of the fluidized bed partially roasted particles of ore finer than about 100 mesh, passing the suspension of partially roasted feed ore in gas from the top of the bed into a free space thereabove having a height ten to twenty times the height of the fluidized bed, passing the partially roasted ore suspended in the gas through the free space to effect substantially complete oxidation of the sulfide ore to the corresponding oxide, maintaining the temperature of the free space thereabove within the range of 1600-1750° F., controlling the temperature of the fluid bed by the introduction of water directly into the fluid bed and the temperature of the free space above the bed by recycling cooler gas into the free space, discharging the substantially completely roasted ore and gas from the free space, separating at least 90 percent of the roasted ore particles from the gas while maintaining a temperature within the range of about 1500-1700° F. prior to and during separation of the roasted ore particles from the gas, discharging the separated roasted particles from the separator, discharging the gas from the separator, cooling the gas by passing it through a waste heat boiler, and recovering the remainder of the fine particles of dust in the gas by passing it through an electrostatic precipitator.

#### References Cited by the Examiner

##### UNITED STATES PATENTS

|           |       |             |       |      |
|-----------|-------|-------------|-------|------|
| 2,847,294 | 8/58  | Long et al. | ----- | 75-9 |
| 2,855,288 | 10/58 | Cyr et al.  | ----- | 75-9 |
| 3,047,365 | 7/62  | Jukkola     | ----- | 75-9 |

##### FOREIGN PATENTS

|         |       |                |
|---------|-------|----------------|
| 482,962 | 5/52  | Canada.        |
| 645,977 | 11/50 | Great Britain. |

70 BENJAMIN HENKIN, Primary Examiner.

DAVID L. RECK, Examiner.